

## UNITED STATES PATENT OFFICE.

WILHELM HELMUT SCHWEITZER, OF HEIDELBERG, GERMANY, ASSIGNEE, BY MESNE ASSIGNMENTS, TO AMERICAN LANIL CORPORATION, A CORPORATION OF NEW JERSEY.

## MANUFACTURE OF TEXTILE FIBERS FROM ANIMAL HAIR AND BRISTLES.

No Drawing. Application filed November 17, 1922, Serial No. 601,646, and in Germany February 13, 1922.

A known manufacture of textile fibers from animal hair and bristles consists in treating the material with chlorinating or oxidizing agents and then subjecting the 5 chlorinated or oxidized fibers to subsequent treatment with soap and soluble oils, or with agents having an alkaline reaction; for the latter subsequent treatment it has hitherto been the rule to use a large excess 10 of alkali. In the preferred process, the chlorinating or oxidizing agent is used in proportion which exceeds 12 per cent of the weight of the material in the case of chloride of lime and in the case of chlorine 25 litres 15 of the gas to 1 kilo of the material.

The present invention relates to the manufacture of textile fibers from animal hair and bristles by treatment of the chlorinated or oxidized fibers with alkali, but differs 20 from the processes hitherto proposed in that the alkali or the alkaline agent for the subsequent treatment of the fibers is used only in such proportion that only a distinct alkaline reaction is produced. After this 25 treatment the fibers may be washed, dried, or in some cases, treated with soap or soluble oils in known manner.

The following example illustrates the invention:

30 100 kilos of cross bred cardings are oxidized by means of a cold acidified filtered solution from 100 kilos of chloride of lime for about half an hour and are then well washed.

35 The cardings are then passed through a cold bath consisting of a caustic soda solution containing 0.1 to 0.15 gram of caustic soda per 100 cc. of water, 30 litres of the bath being used per kilo of fiber. After this treatment follow two washing baths.

The goods may then be dried on heated cylinders.

The essence of the invention is the use of a small excess of alkali. When a solution of caustic soda of 1 per cent strength, for example, acts upon oxidized animal fibers, the easily soluble albumin bodies pass into solution and are afterwards washed away; by this invention, however, this does not happen as the alkali is consumed in forming 45 a salt. Thus by the invention the dissolution of albumin bodies is avoided and the oxidized material suffers much less loss of 50 weight than in the known processes.

What I claim is:

1. A process for the production of animal fibers suitable for use in the production of textile fabrics, which consists in taking animal fibers which have been oxidized and subjecting the same to a bath of caustic soda 60 solution from 0.1% to 0.15% in strength and sufficient to form an alkaline salt upon the fibers whilst insufficient in strength to dissolve the albumin bodies present therein, washing the thus treated fibers and drying 65 the same.

2. The process of treating oxidized or chlorinated animal fibers to produce textile fibers, which consists in passing the fibers through a caustic soda solution containing 70 0.1 to 0.15 grams of caustic soda per 100 cc. of water, approximately 30 litres of the bath being used per kilo of fiber, thence washing the treated fiber and drying the same.

In witness whereof I have hereunto signed 75 my name this 2nd day of November 1922.

WILHELM HELMUT SCHWEITZER.